



US008986817B2

(12) **United States Patent**  
**Wang et al.**

(10) **Patent No.:** **US 8,986,817 B2**  
(45) **Date of Patent:** **Mar. 24, 2015**

(54) **NITRIDED COMPONENT SURFACE REPAIR**

(71) Applicant: **Caterpillar Inc.**, Peoria, IL (US)

(72) Inventors: **Huijun Wang**, Peoria, IL (US); **Marion B. Grant**, Princeville, IL (US)

(73) Assignee: **Caterpillar Inc.**, Peoria, IL (US)

(\*) Notice: Subject to any disclaimer, the term of this patent is extended or adjusted under 35 U.S.C. 154(b) by 28 days.

(21) Appl. No.: **13/795,044**

(22) Filed: **Mar. 12, 2013**

(65) **Prior Publication Data**

US 2014/0272323 A1 Sep. 18, 2014

(51) **Int. Cl.**

**B32B 3/00** (2006.01)

**C25B 11/04** (2006.01)

**F02M 59/44** (2006.01)

**F02M 59/48** (2006.01)

(52) **U.S. Cl.**

CPC ..... **C25B 11/0478** (2013.01); **F02M 59/44** (2013.01); **F02M 59/48** (2013.01); **F02M 2200/80** (2013.01); **F02M 2200/9038** (2013.01)

USPC ..... **428/195.1**; 428/209; 427/142

(58) **Field of Classification Search**

CPC ..... C23C 18/1605; C23C 18/1637; C23C 18/1692; B32B 15/01

USPC ..... 428/195.1, 209; 427/142

See application file for complete search history.

(56) **References Cited**

U.S. PATENT DOCUMENTS

4,358,922 A \* 11/1982 Feldstein ..... 57/401  
4,636,255 A 1/1987 Tsuda et al.  
2002/0045053 A1 \* 4/2002 Hoskin ..... 428/469  
2011/0206532 A1 8/2011 Sorbo et al.

FOREIGN PATENT DOCUMENTS

JP 2011174181 A 9/2011

\* cited by examiner

*Primary Examiner* — Elizabeth Mulvaney

(74) *Attorney, Agent, or Firm* — Finnegan, Henderson, Farabow, Garrett & Dunner, LLP

(57) **ABSTRACT**

A plunger for fuel injection assembly is provided. The plunger includes a nitrided surface. The nitrided surface includes a damaged area. An electroless material is coated on the damaged area.

**20 Claims, 5 Drawing Sheets**





FIG. 1



FIG. 2



FIG. 3





## NITRIDED COMPONENT SURFACE REPAIR

## TECHNICAL FIELD

The present disclosure relates to a method for repairing a damaged surface and more particularly to repairing of a hardened surface of a machine component.

## BACKGROUND

Electroless metal coatings on machine components for enhanced performance are known in the art. The electroless coating process is typically used for enriching the surface of metallic components for protection against corrosion, wear, etc. For example, U.S. Published Application No. 2011/206532 relates to an electroless coating process including coating a substrate with an electroless coating and then heating to a specific temperature.

Some engines are assembled with surface hardened components. A nitriding process is widely used for surface hardening of the components. The nitriding process is a heat treatment process that diffuses nitrogen into the surface of the metallic component to create a case hardened surface. The component may be made from steel, iron, titanium, and the like. The component that is subjected to the nitriding process may already be in a hardened and tempered condition. This may allow for the nitriding process to take place at a temperature lower than the last tempering temperature. Further surface treatment, such as, for example, coating or cladding, may be conducted at a lower temperature than that of the nitriding temperature, in order to avoid damaging of the nitride hardened layer.

During operation, the nitrided surface of the component may be subjected to wear, cavitation, erosion, tear, corrosion, or other damage. The damage may be due to the application of higher force, surface strain, torsion, bending moment, or other environmental conditions. Damages to the nitrided surface may result in unsatisfactory performance, sometimes requiring replacement of the parts with new components. This may lead to an overall increase in costs.

Various methods for repairing these damaged components are known in the art. For example, micro arc welding and laser beam cladding can be used for coating a material on the nitrided surface. However, these techniques are thermal based repair processes that may damage a base material strength of the nitrided surface. High temperatures involved in thermal based repair processes can lead to out-gassing of nitrogen from the nitrided surface, causing a reduction in the hardness of the nitrided surface. The out-gassing of nitrogen may also lead to porosity issues in the coated material.

Other known techniques include chrome plating and High Velocity Fuel Oxygen (HVOF). However, the chrome plating technique is not environment friendly. In the HVOF method, bonding between the coated material and the nitrided surface is not metallurgical, thus affecting the bond strength.

Hence, there is a need of providing an improved method of repair for nitrided components.

## SUMMARY

In one aspect of the disclosure, a plunger for fuel injection includes a nitrided surface. The nitrided surface includes a damaged area and an electroless material coated on the damaged area.

In another aspect of the disclosure, a method includes introducing a nitrided surface having a damaged area for a predetermined time period into a bath containing an electro-

less material. The method also includes coating the damaged area with the electroless material, and heat treating the electroless material at a predetermined temperature for a predefined time.

In yet another aspect, a nitrided surface is provided. The nitrided surface includes a damaged area. An electroless material is coated on the damaged area.

## BRIEF DESCRIPTION OF THE DRAWINGS

10

FIG. 1 is a sectional view of an exemplary fuel injection assembly having a plunger, according to one embodiment of the present disclosure;

15

FIG. 2 is an isometric view of the plunger shown in FIG. 1, a damaged area clearly visible on a nitrided surface of the plunger;

FIG. 3 is an sectional view of an exemplary fuel injector assembly having a poppet;

20

FIG. 4. is an isometric view of the poppet shown in FIG. 3, the damaged area clearly visible on the nitrided surface of the poppet; and

FIG. 5 is a flowchart of an exemplary method for repairing the damaged area on the nitrided surface.

## DETAILED DESCRIPTION

25

Reference will now be made in detail to specific embodiments or features, examples of which are illustrated in the accompanying drawings. Generally, corresponding or similar reference numbers will be used, when possible, to refer to the same or corresponding parts.

30

Referring now to FIG. 1 an exemplary fuel injection assembly 100 of a diesel engine is illustrated. The fuel injection assembly 100 may include a plunger 102 slidably and rotatably placed in a barrel 104. The barrel 104 may be configured to have an inlet port 106 and a spill port 108. The plunger 102 may be configured to rotate and slide in the barrel 104, in order to effectuate substantial delivery of pressurized fuel into a cylinder of the diesel engine at a predetermined time.

35

During operation of fuel injection assembly 100, the barrel 104 may receive a substantial quantity of fuel through the inlet port 106. Thereafter, the plunger 102 may compress the fuel in the barrel 104 in order to increase the pressure of the fuel. The high pressure fuel from the barrel 104 may then be introduced into a connector portion 114 through a delivery valve 110. The delivery valve 110 is located within an outlet portion 112 of the fuel injection assembly 100. Further, the connector portion 114 may deliver the high pressure fuel to an injector (not shown) in order to inject the fuel into the cylinder. The spill port 108 may be configured to provide the additional fuel in the barrel back to a fuel tank.

40

FIG. 2 illustrates the plunger 102 utilized in the fuel injection assembly 100, according to various embodiments of the present disclosure. The plunger 102 has an outer surface 202 including an upper portion 204, a middle portion 206 and a lower portion 208. As illustrated in FIG. 1, the upper portion 204 may be in fluid communication with the fuel in the barrel 104 of the fuel injection assembly 100 for discharging a specific amount of fuel at a predetermined time. The middle portion 206 of the plunger 102 may be in contact with an inner wall of the barrel 104 of the fuel injection assembly 100. The lower portion 208 of the plunger 102 may include an integrated gear segment 210.

45

Another exemplary machine component is depicted in FIGS. 3 and 4. FIG. 3 illustrates a fuel injector assembly 300 utilized in connection with the diesel engine. The fuel injector assembly 300 may include a first portion 302, an intermediate

portion 304 and a nozzle portion 306. The first portion 302 may include a poppet 308 and a plurality of passages 310. The intermediate portion 304 may include a passage 312. The intermediate portion 304 may be connected to the first portion 302 and the nozzle portion 306.

During operation, the first portion 302 may receive the pressurized fuel from the fuel injection assembly 100. The first portion 302 of the fuel injector assembly 300 may then deliver the pressurized fuel to the nozzle portion 306 via the passages 312 located within the intermediate portion 304 and the passages 310 of the first portion 302. Thereafter, the nozzle portion 306 may inject the pressurized fuel in the cylinder of the diesel engine.

FIG. 4 illustrates the poppet 308 utilized in the fuel injector assembly 300. The poppet 308 has the outer surface 202 including an upper portion 402, a tapered middle portion 404, and a lower portion 406. As shown in FIG. 3, the upper portion 402 of the poppet 308 may be in contact with the passage 310 of the first portion 302. The tapered middle portion 404 at one end is in contact with an internal wall of the first portion 302 and at other end is in contact with a spring 314 located within the first portion 302. Further, the lower portion 406 of the poppet 308 may be connected to an external cap 316 of the fuel injector assembly 300.

The plunger 102 and/or the poppet 308 may be made of a metal. In some embodiments the metal may include an alloy of steel, iron, or titanium. Other embodiments may include any metal known in the art. The outer surface 202 of the plunger 102 and/or the poppet 308 may be hardened by a surface treatment process, such as, but not limited to, a nitriding treatment process. The nitriding treatment process involves diffusing nitrogen into a base material at high temperatures. The high temperatures may include a range of 550-590° C. to provide the required surface hardness.

In one embodiment, during the operation of the fuel injection assembly 100, the plunger 102 may be damaged due to contact with other components in the fuel injection assembly 100. This damage on the nitrided surface 202 may be caused by a variety of factors including cavitation, erosion, corrosion, wear and tear, and/or higher forces. For example, the middle portion 206 of the plunger 102 may be damaged due to contact with the inner wall of the barrel 104 of the fuel injection assembly 100. In another example, increased fuel injection pressure within the barrel 104 may cause cavitation damage on the plunger 102. Usually, the cavitation damage is similar to scars, shown as the on the damaged area 212 in FIG. 2. The scar may have a depth of up to 150 micrometer.

During the operation of the fuel injector assembly 300, the poppet 308 may be exposed to damage due to contact with other components of the fuel injector assembly 300. For example, a surface of the tapered middle portion 404 of the poppet 308 may be damaged due to contact with the inner wall of the first portion 302. In another example, increased friction between the surface of the tapered middle portion 404 and inner wall of first portion 302 as well as abrupt changes in fuel pressure may cause cavitation and/or erosion damage on the poppet 308. The exemplary damaged area 212 on the poppet 308 is shown in the FIG. 4. As described earlier, the damaged area 212 on the nitrided surface 202 of the plunger 102 and/or the poppet 308 may include, for example, scratch marks, scars, deformations, abrasion marks, and erosion marks. A person of ordinary skill in the art will appreciate that the location, type and extent of damage described herein is exemplary.

FIG. 5 depicts a method 500 for repairing the damaged area 212 on the nitrided surface 202 of the plunger 102 and/or poppet 308. The damaged area 212 on the nitrided surface 202

is coated with an electroless material. The electroless material may include nickel (Ni), phosphorus (P), boron (B), or any combination thereof. For example, the electroless material may be a solution of nickel (Ni) with high phosphorus (P) content. One of ordinary skill in the art will appreciate that the electroless solution of nickel (Ni) with high phosphorus (P) content may result in a coated surface with a relatively higher surface hardness.

The coating of the electroless material on the nitrided surface 202 is configured to provide a surface hardness in a range of approximately 60-70 HRC. Known electroless Ni coating has plated hardness values in a range a range of approximately 49-62 HRC. These hardness values can be increased to approximately 64-70 HRC on heat treatment. It should be understood that surface hardness in the approximate range of approximately 60-70 HRC is desirable on the machine components, in order to provide protection from wear and tear that these components may undergo during operation.

A method 500 for repairing the nitrided surface 202 will be further described in detail in connection with FIG. 5.

#### INDUSTRIAL APPLICABILITY

The fuel injection assembly plunger 102 and/or the poppet 308 of the fuel injector assembly 300 may be subjected to damage during operation. The damage may result in unsatisfactory overall performance of the plunger 102 and/or the poppet 308. One solution includes replacing the plunger 102 and/or the poppet 308 by a new one. However this solution poses cost considerations. Other approaches include repairing the damaged area 212 on the nitrided surface 202 of the plunger 102 and/or the poppet 308. Many surface repairing methods such as thermal processes, plating processes and other deposition methods are known in the art.

Thermal repairing processes like micro arc welding, laser beam cladding, etc. may have an effect on surface properties of the repaired surface. During the nitriding process, nitrogen gas is diffused into the surface of the base material, to form a coated base material. The base materials used in the manufacture of the machine components include steel, iron, titanium, and the like. The thermal processes are carried at relatively higher temperatures, causing the out-gassing of nitrogen from the coated base material.

For example, in laser or welding based cladding processes, due to high heat input from the cladding processes the temperature attained at the coated base material is higher than the temperature at which nitriding process is performed. As a consequence, the diffused nitrogen is released from the coated base material, leading to the formation of pores. This may reduce the surface hardness of the base material nitrided surface and also cause porosity in the coated layer.

Further, the known plating process, such as chrome plating, may provide a surface with relatively lesser hardness. This may be undesirable due to the harsh working environment conditions that the machine components are generally subjected to. The lesser hardness may impact the tendency of these components of being susceptible to damage. Other deposition processes like HVOF provide negligible metallurgical bonding between the coating and the base material.

The present disclosure relates to the method 500 of repairing the damaged area 212 on the nitrided surface 202 of the plunger 102 and/or the poppet 308 by using electroless process. The method 500 may be carried out at relatively lower temperatures, preventing the out-gassing of nitrogen from the nitrided surface 202. Additionally, the method 500 does not require electric current, resulting in uniform and continuous coating on the nitrided surface 202. The electroless coating

may provide a relatively high bond strength of about 40,000-60,000 psi on steel. Further, the method 500 provides for the resultant surface hardness in a range of approximately 60-70 HRC. This may be a desired hardness required for the machine component to be less susceptible to damage.

FIG. 5 shows the method 500 for repairing the nitrided surface 202. Initially at step 502, the nitrided surface 202 of the plunger 102 and/or the poppet 308 having the damaged area 212 may be subjected to a pre-treatment process. During pre-treatment, the nitrided surface 202 may be cleaned by any standard cleaning process known in the art. This cleaning process may be washing, polishing, precision grinding, wiping, rinsing, chemical treatment or any combination thereof. For example, the damaged area 212 may be precision ground with a tool like a precision grinding wheel in order to remove any irregularities and level-out the nitrided surface 202.

In one embodiment, remaining areas of the nitrided surface 202 of the plunger 102 and/or the poppet 308, i.e. damage-free areas or areas which do not require coating, may be masked or covered with a polymer mask or any other suitable material mask. The masking may involve tying of a cloth or a polymeric sheet on exposed areas of the nitrided surface 202 by mechanical fasteners like bands, on a temporary basis, until the method 500 is completed. The masking or covering may prevent deposition of electroless material on the damage-free area.

At step 504, the nitrided surface 202 may be introduced into a bath of an electroless solution containing ionic Nickel and ionic Phosphorus (1% to 13% Phosphorus) for a predetermined period of time. The bath may include an open vessel containing the electroless solution. In other embodiments other electroless solutions may be used as would be known in the art. At step 506, the electroless material may be coated on the damaged area 212. It should be noted that the predetermined period of time for which the nitrided surface 202 is held in the electroless solution may depend on a thickness of the coating required on the damaged area 212.

During the electroless Nickel coating at step 506, the coating process auto-catalytically deposits Nickel alloyed with Phosphorus (12% by weight) on the nitrided surface 202. For example, electroless nickel coating using sodium hypophosphate as the reducing agent proceeds via the following overall reduction/oxidation reaction:



At step 508, the nitrided surface 202 may be subjected to heat treatment. The heat treatment may increase the hardness imparted by the electroless material on the nitrided surface 202, resulting in hardness of approximately 60 to 70 HRC. In an exemplary case, heat treatment of the nitrided surface 202 of the plunger 102 and/or the poppet 308 may involve baking, wherein there is rise in temperature at the start of the heat treatment and relatively slow decrease in temperature at the end of the heat treatment. This may avoid any micro-cracking in the electroless material coated on the damaged area 212.

The nitrided surface 202 may be heated at a predetermined temperature for a predefined time period. The predetermined temperature at which the nitrided surface 202 is heated is in a range of approximately 200° C. to 400° C. Also, the predefined time for which the nitrided surface 202 is heated lies may be less than 24 hours. One of ordinary skill in the art will appreciate that the predetermined temperature and the predefined time should be selected in such a way that the properties of the nitrided surface 202 is subjected to minimal or no change. More importantly, the predetermined temperature

should be low enough in order to prevent the out-gassing of nitrogen from the nitrided surface 202.

At step 510, the nitrided surface 202 may be subjected to machining, wherein after the heat treatment, one or more dimensions of the resultant surface are processed to achieve desired engineering standards. The engineering standards may be engineering dimensions, surface finish, or any other standard which is necessary for the plunger 102 and/or the poppet 308 being repaired to function in the respective working environment. The machining process could be any standard machining process known in the art. The machining process may include polishing, precision grinding, turning, or any other method known in the art.

The present disclosure has been explained with reference to the damaged area 212 present on the plunger 102 and/or the poppet 308. However, the present disclosure does not restrict itself to the nitrided fuel injection plunger 102 and/or the nitrided poppet 308. The nitrided component can include any nitrided element that may be used in standard automobile engine applications.

While aspects of the present disclosure have been particularly shown and described with reference to the embodiments above, it will be understood by those skilled in the art that various additional embodiments may be contemplated by the modification of the disclosed machines, systems and methods without departing from the spirit and scope of what is disclosed. Such embodiments should be understood to fall within the scope of the present disclosure as determined based upon the claims and any equivalents thereof.

What is claimed is:

1. A plunger for a fuel injection assembly, the plunger comprising:  
an outer nitrided surface having a first hardness, the outer nitrided surface including at least one damaged area; and an electroless material coated on the damaged area, the electroless material having a second hardness different from the first hardness.
2. The plunger of claim 1, wherein the second hardness ranges between 60 and 70 HRC.
3. The plunger of claim 1, wherein the electroless material includes a least one of nickel and phosphorus.
4. The plunger of claim 1, wherein the damaged area includes cavitation damage.
5. A method for repairing a nitrided surface having a damaged area, the method comprising:  
introducing the nitrided surface into a bath containing electroless material for a predetermined period of time;  
coating the damaged area with the electroless material;  
heat treating the electroless material at a predetermined temperature for a predefined time, the predetermined temperature being selected to prevent outgassing of nitrogen from the nitrided surface.
6. The method of claim 5, wherein the electroless material is configured to provide surface hardness between 60 and 70 HRC.
7. The method of claim 5, wherein the electroless material includes at least one of nickel and phosphorus.
8. The method of claim 5 further comprising pre-treating the nitrided surface.
9. The method of claim 5 further comprising covering a damage-free area of the nitrided surface prior to the introduction of the nitrided surface into the bath.
10. The method of claim 5 further comprising machining the electroless material to a desired finish after the heat treating.

11. The method of claim 5, wherein the pre-determined period of time for the introduction of the nitrided surface into the bath is based on a thickness requirement of the electroless material.

12. The method of claim 5, wherein the predetermined temperature for the heat treating lies in a range between 290 and 400° C. 5

13. The method of claim 5, wherein the predefined time for the heat treating is less than 24 hours.

14. The method of claim 5, wherein the nitrided surface 10 includes at least a portion of a plunger for a fuel injection assembly.

15. The method of claim 14, wherein the damaged area includes cavitation damage on the plunger.

16. A nitrided surface comprising: 15  
an undamaged area having a first hardness;  
at least one damaged area; and  
an electroless material coated on the damaged area of the  
nitrided surface, the electroless material having a second  
hardness different from the first hardness. 20

17. The nitrided surface of claim 16, wherein the second hardness ranges between 60 and 70 HRC.

18. The nitrided surface of claim 16, wherein the electro- 25  
less material includes a least one of nickel and phosphorus.

19. The nitrided surface of claim 16, wherein the nitrided 25  
surface includes at least a portion of a plunger of a fuel  
injection assembly.

20. The nitrided surface of claim 16, wherein the damaged area includes cavitation damage on the plunger.

\* \* \* \* \*

30